

May 9, 1944.

G. J. D'EUSTACHIO

2,348,333

LEAD ALLOY

Filed March 29, 1941

2 Sheets-Sheet 1



Fig. 1.



Fig. 2.



Fig. 3.

INVENTOR

Gabriel Joseph D'Eustachio

BY

George J. Schotteler

ATTORNEY

May 9, 1944.

G. J. D'EUSTACHIO

2,348,333

LEAD ALLOY

Filed March 29, 1941

2 Sheets-Sheet 2



Fig. 4.



Fig. 5.



Fig. 6.

INVENTOR

Gabriel Joseph D'Eustachio

BY

George J. Schreier

ATTORNEY

## UNITED STATES PATENT OFFICE

2,348,333

## LEAD ALLOY

Gabriel Joseph D'Eustachio, Perth Amboy, N. J.,  
assignor to General Cable Corporation, New  
York, N. Y., a corporation of New Jersey

Application March 29, 1941, Serial No. 385,884

8 Claims. (Cl. 75—166)

This invention relates to extruded metal cable sheaths and to lead base alloys suitable therefor, and has for an object the provision of an improved alloy for this purpose.

When subjected to stresses, lead has a tendency to deform slowly or to "creep." Even stresses which are only a fraction of those required to develop the short-time breaking strength will cause creep when applied for long periods of time. As examples of stresses which may cause creep in the lead sheath of cables, there may be mentioned the fairly constant internal pressures of oil-filled cables and the varying pressures of solid type cables caused by the combination of hydraulic head and volume change due to temperature cycles. Lead sheaths are also subject to fatigue under cyclic stresses.

It has long been known that the inclusion of some other metal with lead may produce an alloy of greater strength than lead alone and that extruded sheaths of some of these alloys have greater fatigue resistance and less tendency to creep than sheaths of lead alone. For example, lead may be alloyed with copper and the resulting material used as a cable sheath. The amount of copper so used is usually 0.06%, or less, since a larger amount of copper than this cannot remain in solution in lead when the alloy is cooled to the freezing point. A sheath made of such an alloy is much superior to a sheath composed of pure lead, both in respect to fatigue resistance and to flow or creep.

When this alloy cools to room temperature, only about 0.02% copper remains in solution in lead, the remaining approximately 0.04% being segregated in the mixture. Certain difficulties are encountered in the use of this binary lead-copper alloy, especially for cable sheaths, which, in some instances, more than offset its beneficial properties. The undesirable properties result from the uneven segregation, aggregation or concentration of copper particles in certain portions of the mass, these portions being at or near the welds, tongues and flow lines in the finished sheath. The presence of the excess amount of copper in these regions results in an embrittlement and weakness in the finished sheath.

Even with pure or "common" lead, which is a commercial lead of high purity, these welds, tongues and flow lines are regions of weakness unless refined methods of lead press operation are used to overcome the difficulties encountered with older practices. The use of the vacuum lead press process is one method of reducing or eliminating these difficulties with common lead.

However, in the case of copper-bearing lead, even sheaths extruded on the vacuum press have, to a degree, this weakness at welds, tongues and flow lines resulting from the segregation of the copper content and its aggregation or concentration at these points.

This uneven distribution of the copper content is most clearly shown by special etching methods which do not dissolve the copper particles but change them to copper oxide which appears as a black deposit. Sections of the binary lead-copper alloy which have been etched according to this procedure show a heavy black deposit of copper oxide in the region of the welds, tongues and flow lines. This characteristic of the etched surface has not commonly been observed because the etching methods which are in most general use either remove the copper from the etched surface or do not leave it in the readily visible form resulting from this etching procedure.

A slight variation of the etching procedure, designed to bring out the grain structure in the same sections, reveals groups of grains of much smaller size than in the major portion of the cross section.

The disadvantage to practical service due to the weakness produced by this uneven segregation, aggregation or concentration of copper in the regions of the welds, tongues and flow lines is shown by the results of an extensive series of tests in which cable sheaths of various types were subjected to internal hydrostatic pressure.

Tests in one series, extending over a period of a few days, which may be referred to as short-term tests, were performed on tightly sealed cables in which electric current was circulated in the conductors to heat them. This resulted in heating and expansion of the saturant and, in turn, in increased pressure on the sheath. The rate of heating was so controlled that the internal hydrostatic pressure as measured by a gauge did not exceed 100 to 125 lbs. per sq. in., corresponding to a fiber stress in the sheath of about 1000 to 1200 lbs. per sq. in. As the sheath stretched, the current was increased but limited to a value producing a conductor temperature of 95° C., the corresponding sheath temperature being 75 to 80° C. In the case of sheaths formed of common lead, the sheath stretched sufficiently to take care of the expansion and no rupture resulted; but in the case of lead-copper sheaths, rupture did occur in a large proportion of specimens, the rupture taking the form of longitudinal slits along the weld regions.

According to the present invention, the difficult

ties encountered with these binary alloys of lead and copper are overcome by the inclusion of a third metal which is mutually soluble with either of the first two metals. For example, tin may be used because it satisfies these conditions and produces excellent results.

Tin has been found to produce good results when added in amounts of from 0.03% to 0.5%. Most of the benefits are obtained with amounts of from 0.06% to 0.12%. Ordinarily, because no further pronounced benefits are obtained and because of the increase in cost, amounts greater than 0.12% are not used. If amounts in excess of 0.5% are used, this results in gradually reduced creep strength, though up to 3% is not particularly harmful. In the other direction, definite benefits are found with amounts as low as 0.03%, and some benefits with even less.

As an example, for a lead base copper alloy containing 0.06% copper, good results were obtained with a tin content of 0.06% to 0.12%, as shown by test data hereinbelow.

Where the binary lead-copper alloy is used, it is the common practice to use the full 0.06% copper which is retained in solution at the melting point of the alloy, because the beneficial effect of the copper addition falls off rapidly with smaller amounts. However, when tin is included in a ternary alloy of lead-copper-tin, the effects of the tin are such that a useful product will result, even where copper is present in amounts less than 0.06%, say 0.03%, simply retaining whatever valuable properties may be imparted by such amounts of copper as are used. On the other hand, the use of tin makes it practical to use more than 0.06% copper, up to 0.08% copper having been found permissible. For any amount of copper within this range, the amount of tin to be used falls within the same range as for 0.06% copper.

Tests and observations have shown that concentration of copper along tongues, flow lines and welds which characterizes the binary alloy is substantially absent in the ternary alloy of the present invention. This may be seen in the accompanying drawings, wherein:

Fig. 1 is a photomicrograph at 12 diameter magnification of one of the weld regions of a cable sheath formed of a binary alloy containing 0.06% copper and the balance lead. The sample was etched for detection of copper segregation. The black regions 10 represent the excess copper and 11 indicates the weld.

Fig. 2 is a photomicrograph at the same magnification and of the same binary alloy etched in the same way as in Fig. 1, but taken in the region of the tongues and flow lines. The black regions at the boundaries of the tongues where copper aggregation occurs is indicated by the numeral 12.

Fig. 3 is a photomicrograph at the same magnification and of the same binary alloy as in Fig. 1, but etched and treated to bring out the grain structure in the tongue region, such as that shown in Fig. 2. During etching, the specimen was swabbed to remove the copper oxide and consequently the black areas are absent. The microstructure reveals a concentration of very minute grains at the boundaries of the tongues, as indicated at 12a.

Fig. 4 is a photomicrograph at the same magnification of a ternary alloy containing 0.06% copper, 0.06% tin, and the balance lead, the section being taken in one of the weld regions and prepared in the same way as that of Fig. 1. It is to be noted that there are no black regions of

copper oxide in Fig. 3, nor is there a film of copper oxide to make the surface indistinct as in Fig. 1; but, on the contrary, the grain structure is distinct, as in Fig. 3 where the specimen was swabbed, though the Fig. 4 specimen was not swabbed. The weld line is faintly indicated at 11'. Grain formation across the weld line is even indicated. When such specimens are swabbed, the weld lines are still more faint.

Fig. 5 is a photomicrograph at the same magnification and of the same ternary alloy as in Fig. 4, but taken in the tongue region and the section prepared in the same way as that of Fig. 2. It was only by careful etching and search that the section was located, even when inspecting the dimensionally charted areas where tongues were usually found. The tongue 15 is shown only by a very slight shadow or darkening, and the boundaries of the tongue show no distinction whatever in grain structure from the other areas.

Fig. 6 is a photomicrograph at the same magnification and of the same specimen as that shown in Fig. 5 but etched and swabbed like the binary specimen of Fig. 3 to bring out the grain structure in the tongue region for comparison with the same region in the binary alloy sheath shown in Fig. 3. The view would appear substantially the same if it had not been swabbed, because of the absence of copper oxide. It is to be noted that the grains are of uniform size throughout and that there is no concentration of small grains, as in Fig. 3.

When specimens of the binary alloy, such as that shown in Figs. 1, 2 and 3, and that of test specimen No. 1 below, were left for several days in old etching solution (essentially lead acetate-acetic acid-alcohol but containing a very small amount of copper in solution), they showed a very thick deposit rich in copper (appearing after treatment as copper oxide) over the entire face, and showed wide black markings of copper oxide at the tongues and welds. The ternary alloys, such as that shown in Figs. 4, 5 and 6, and the test specimens Nos. 2, 3 and 4 below, when similarly treated showed no such surface deposit and only a very slight discoloration.

Except for very slight markings at the welds, as seen in Fig. 4, and the shadings which can with care be produced at the tongues, as seen in Fig. 5, the ternary alloys acquire the same color as commercially pure lead during the etching process. When swabbed, these slight markings disappear and grains of uniform size appear over the entire surface, even across the weld line, as seen in Fig. 6.

In operating an extrusion press to form cable sheaths of the ternary alloy, the desired amount of tin may be added in the melting pot to the molten binary lead-copper alloy; or, if preferred, the ternary lead-copper-tin alloy may be previously formed and supplied to the melting pot as a ternary alloy.

Reference has been made hereinabove to extensive series of tests in which cable sheaths of various types were subjected to internal hydrostatic pressure for various periods of time. In one series, the tests were limited to a predetermined hydrostatic pressure or to a predetermined small amount of expansion as determined by other purposes of the test. In another series, the tests were carried to rupture of the sheath, the time to rupture depending upon the amount of pressure and varying from a few minutes to many months. In another long term group, extending over a period running up to a few years,

the creep characteristics of the alloys were determined by measurements upon strips.

In addition, measurements were made of fatigue strength and also tensile tests were made on strips cut from extruded tubes composed of binary and ternary alloys of the same composition as those from which the accompanying photomicrographs were made, as well as from some other ternary alloys of different tin content. The tensile tests show that the tensile strength of the ternary alloy was definitely in the same range as that of the binary alloy, and in one set of tests it proved somewhat superior, as shown by the following data:

| Alloy No. | Copper  | Tin     | Lead         | Tensile strength |
|-----------|---------|---------|--------------|------------------|
|           | Percent | Percent | Remainder    | p. s. i.         |
| 1.....    | 0.06    | None    | .....        | 2,050            |
| 2.....    | 0.06    | 0.06    | .....do..... | 2,250            |
| 3.....    | 0.06    | 0.12    | .....do..... | 2,270            |
| 4.....    | 0.06    | 0.5     | .....do..... | 2,420            |

On another lot of samples, the difference in tensile strength between the binary and ternary alloys was somewhat less than for the samples of the above tabulation, but a slight difference in favor of the ternary alloy was still indicated.

In the first mentioned series of hydraulic pressure tests—those not intended to be carried to failure—it has been noted that sheaths formed of the binary alloy ruptured with very small elongation occurring in these tests. It is also noted that sheaths formed of common lead stretched the required amount under the same conditions but did not break. Similar tests were also applied to sheath formed of the ternary alloy and reached the full required amount of elongation and did this without failure. It is to be noted that the sheath temperature during these tests was considerably higher than the temperature of the lead pipe in the tests in the following mentioned series which were intentionally carried to failure. Other data have shown that where bursting tests are carried on at high temperature, less elongation occurs before failure on sheath containing lines of weakness, as in the case of the binary alloy. Thus, these binary alloy sheaths, tested at the high temperature, failed with much less elongation than in the long time tests made at lower temperature.

In the series of tests with hydraulic pressure in which the tests were purposely carried on to failure, it was found that sheath formed of the binary alloy behaved entirely differently on the short time and on the long time tests. For the test of less than 7 days' duration, an elongation of approximately 20% was obtained and the breaks were wedge-shaped or gradual, that is, attenuated or drawn out. Wedge-type ruptures are recognized as being characteristic of homogeneous metal structures, whereas blunt ruptures indicate non-homogeneous zones. For tests at lower pressures which extended for more than 7 days, the elongation was less, decreasing as the length of the test increased and the failures were radial or abrupt, that is, blunt or almost perpendicular to the wall. On the other hand, all of the ruptures in the ternary alloy sheaths were wedge-shaped. Also, the elongation on the ternary alloy was as great on the long time as on the short time test and always in the same range as the elongation on the short time test with the binary alloy. Up to the point

at which the binary alloy sheaths failed, the ternary alloy sheaths showed the same range of elongation. The eventual elongation of the ternary alloy sheaths was greater because they took longer to fail and the elongation increased rapidly as the sheaths became progressively more attenuated in the final stages.

Long term tests were made upon strips cut from tubing to determine relative creep resistance of sheaths formed of the ternary alloy as compared with sheaths formed of the binary alloy. For a broad basis of comparison, strips of common lead were also included in the tests. In these tests constant tension was applied to each specimen and the rate of elongation over various periods was measured. The results showed that the ternary alloy had a creep rate in the same range as that of the binary alloy—actually somewhat lower than that of the binary alloy. Otherwise expressed, the creep resistance of the ternary alloy is as good or better than that of the binary alloy, both being in a range far above that of common lead. The test data, showing the creep rate in percent increase in length per year for different applied tensile stresses, are as follows:

| 30                                      | Stress in lbs./sq. in. (p. s. i.) |     |      |     |
|-----------------------------------------|-----------------------------------|-----|------|-----|
|                                         | 200                               | 300 | 400  | 500 |
| CREEP RATE IN PERCENT PER YEAR INCREASE |                                   |     |      |     |
| 35                                      | Common lead.....                  | 1.4 | 12.3 | 50  |

On fatigue test with the rotating beam method on extruded metal, the maximum stress below failure at 20 million cycles was about 700 p. s. i. for either alloy and about 375 p. s. i. for lead.

Corrosion tests of critical sections of the binary and ternary alloys revealed considerable pitting in the binary alloy sheath and much less pitting in the ternary alloy sheath.

No theory is proposed as to the internal condition of the alloy nor the technical physico-chemical phenomena of mutual solubility, miscibility, melting point, and the like, to explain the reasons for the improvement produced by the inclusion of the third metal. It may be regarded merely as a modifying agent which alters the grain size and microstructure in general (flow lines and tongues) and changes the distribution of the insoluble phase (copper). It is sufficient to know that improvement is in fact produced and how it is accomplished.

While it is believed that those skilled in the art readily recognize the terms "tongues," "flow-lines" and "welds" as applied to cable sheaths, it may be explained for the benefit of those less familiar with the art that tongues and flow lines represent boundary surfaces, generally between successive charges of metal in the press; and welds may represent the same thing or may represent the reuniting surfaces or seams beyond the structures which support the core piece in the press. Tongues and flow lines may be regarded as a part of the charge-weld junction produced between successive charges of metal as distorted and modified during extrusion. With a continuous extrusion press, such as is used in certain special cases, the charge welds will no

be present, but the longitudinal seams or weld lines will always be present.

It will thus be seen that the invention provides a ternary alloy which produces a cable sheath having creep strength and fatigue resistance equal to or greater than that of a binary lead-copper alloy but which at the same time has an improved structure free from localized weakness.

When lead is referred to herein, it will be understood that lead of commercial purity is intended. This may contain small amounts of certain other metals. Some of these impurities may be present in the same range as the copper and tin, but since they have no material effect upon the character of the alloy for present purposes, they need not be considered. The copper itself may be wholly or partly present as an impurity in certain types of lead, and to the extent it is present it need not be added.

It is to be understood that the invention may have various embodiments within the scope of the subjoined claims.

I claim as my invention:

1. An extruded cable sheath formed of a lead base alloy containing copper in amounts sufficient to improve resistance to creep and fatigue but not sufficient to prevent extrusion, characterized by the inclusion of tin in amounts ranging from equal to that of the copper up to less than .5% of the alloy for suppressing aggregation of copper at the tongues and flow lines without impairment of the creep strength and fatigue resistance of the alloy and the balance lead with usual commercial impurities.

2. An extruded cable sheath formed of a lead base alloy, composed of copper in amounts between 0.03% and 0.08%, tin in amounts between 0.03% and less than 0.5%, and the balance all lead with usual commercial impurities.

3. An extruded cable sheath formed of a lead base alloy, comprising about 0.06% copper, between about 0.06% and 0.12% tin, and the balance approximately all lead.

5 4. An extruded cable sheath formed of a lead base alloy in which copper is included in amounts sufficient to improve resistance to creep and fatigue, characterized by the inclusion of tin in amounts approximately equal to the amounts 10 of copper for suppressing aggregation of copper at the tongues and flow lines without impairment of the creep strength and fatigue resistance of the alloy.

5 5. An extruded cable sheath formed of an 15 alloy composed of lead and approximately 0.06% copper and tin within a range from about 0.03% to less than 0.5%, characterized by homogeneous uniform grain structure and absence of copper concentration at the tongues, flow lines and 20 welds, and having mechanical properties, such as tensile strength and resistance to creep and fatigue in the same range as those of the same alloy without tin.

6. An alloy suitable for forming extruded cable 25 sheaths and the like, comprising copper in amounts between 0.03% and 0.08%, tin in amounts between 0.03% and less than 0.5%, and the balance all lead with usual commercial impurities.

30 7. An alloy suitable for forming extruded cable sheaths and the like, comprising copper about 0.06%, tin between about 0.06% and 0.12%, and the balance approximately all lead.

8. An alloy suitable for forming extruded cable 35 sheaths and the like, comprising copper about 0.06%, tin about 0.06%, and the balance principally lead.

GABRIEL JOSEPH D'EUSTACHIO.